

April 20, 1954

I. J. NOVAK  
PROTECTION OF DISPERSED ASBESTOS  
FIBERS ON PAPERMAKING MACHINES  
Filed Sept. 10, 1949

2,675,745



Inventor:  
Izador J. Novak  
By Lee J. Gary Atty.

## UNITED STATES PATENT OFFICE

2,675,745

PROTECTION OF DISPERSED ASBESTOS  
FIBERS ON PAPERMAKING MACHINESIzador J. Novak, Trumbull, Conn., assignor to  
Raybestos-Manhattan, Inc., Passaic, N. J., a  
corporation of New Jersey

Application September 10, 1949, Serial No. 114,949

5 Claims. (Cl. 92—38)

1

This invention relates to improvements in the production of felted sheets or webs of fibrous asbestos with generally conventional paper-making apparatus when employing slurries of individualized and dispersed asbestos produced in accordance with my co-pending application, Ser. No. 66,552, filed December 21, 1948, now Patent No. 2,626,213.

More particularly, the present invention relates to the maintenance and protection of the asbestos fibers in such dispersed condition, as distinguished from a flocked or clotted condition while on the foraminous or porous forming or conveying components of the paper-making machine, such as the Fourdrinier wire or felts thereof.

As more fully described in my aforesaid co-pending application, the asbestos dispersions with which the present invention is concerned are prepared by opening and individualizing the fibers of Chrysotile asbestos by subjecting macroscopic bundles or agglomerates thereof (which terms are intended to include mechanically fiberized asbestos) to mild mechanical action, such as stirring or agitation, while immersed in water containing an organic detergent surface-active material adsorbable on the asbestos and capable of forming an alkaline dispersion therewith, the amount of detergent being in excess of that adsorbed on the asbestos and sufficient to form and preserve or maintain the dispersion in a stable manner. Typical examples of such dispersing agents are Aerosol OT (dioctyl sodium sulfosuccinate), sodium oleate, and others more fully particularized in my said co-pending application. Treatment of the asbestos in this manner causes separation, individualization, dissemination and unclotting of the asbestos fibers, and converts them to single fibers or fascicular fiber bundles instead of the predominantly clotted and tangled multiple fiber groups known to prior wet or dry asbestos practice. The fibers in such dispersion are in a lubricated, slippery, relatively slideable condition and composed predominantly of asbestos fibers of "unit size," or "fibro-colloidal diameter," that is, of a diameter of from about 200 to about 500 Angstrom units.

As further set forth in my aforesaid co-pending application, for each surface-active agent, there appears to be a minimum proportion which is adsorbed on the asbestos and therefore required for opening up the asbestos and this must be supplied by using an adequate volume of adequately concentrated agent. However, in addition to the minimum amount required and adsorbed by the asbestos, a further concentration should remain

2

in the liquid for the purpose of dispersing the previously opened fibers. Thus, I have found that beyond the amount necessary to satisfy the fibers, a certain concentration of the agent in the liquid phase is necessary to maintain a stable dispersion. As further described and illustrated in my aforesaid co-pending application, the concentration of the agent in the aqueous phase necessary to maintain the asbestos dispersion over and beyond that which is adsorbed by the asbestos is in the case of Aerosol OT about .035% and for sodium oleate is .047%. These dispersions act in many respects like emulsions or dispersions of other substances in that even though a dispersion may contain an excess of dispersing agent in the liquid phase, dilution thereof by plain water in a rapid manner may cause precipitation or flocculation of the fibers. Further, the addition of water in an amount so as to reduce the concentration of the protective agent or minimum amount required for dispersion will cause flocculation or precipitation of the fibers. As is evident from the foregoing, these surface-active agents are actually colloidizing agents for asbestos in an aqueous vehicle since they reduce the asbestos to colloidal size particles and hold said particles in colloidal dispersion.

An object of the present invention to prevent the shocking of the dispersions employed, and to prevent flocking or precipitation of the fibers on the paper-making machine so as to permit felting of the fibers in their individualized dispersed condition whereby webs or sheets of much greater toughness and flexibility can be produced, as compared to dry webs or sheets composed of heretofore conventional or clotted asbestos fibers. It is a further object of the present invention to prevent clotting or precipitation of dispersed fibers in the paper-making appurtenances such as wires or felts so as to prevent their becoming clotted with asbestos fibers such as, for example, as might occur in carrying out the conventional water washing of a Fourdrinier wire on its return run.

For the purpose of illustration and not limitation, the following is an example of a method for forming an asbestos dispersion, generally described in my aforesaid co-pending application, and the sheeting thereof on a paper-making machine:

A slurry was prepared for making an asbestos tissue by adding 312 lbs. of 25% Aerosol OT in water to 1000 gallons of water and dissolving same therein. Then 212 lbs. of 3R spinning grade Chrysotile asbestos was added and on stirring for

four hours produced a smooth slurry at 2½% asbestos concentration. This was further diluted by adding water slowly to the 2½% slurry in the volume proportion of 9 parts of 2½% slurry to 47 parts water. This produced a smooth ¾% dispersion on mixing for four hours and had a free-ness of 70,000 seconds on a Williams Freeness Tester. The slurry after screening to remove associated impurities, such as serpentine fragments, magnetite inclusions or other clots which do not become softened, was run on a Fourdrinier tissue machine at 85 ft. per minute producing a tissue weighing about 0.7 grams per square foot, having a thickness of about .00035 inch. This tissue was well formed, smooth, uniform in fiber distribution, tough, strong, stretchy, and highly oriented in the machine direction. On its return run the Fourdrinier wire was continuously washed with filtered white water recovered in the operation. In this manner, the screen was continuously freed of the accumulated fibers, clotting of the fibers being prevented therein which might otherwise have occurred had clear water been used for washing. Likewise, had clear water been used for washing sufficient water might have been entrained in or around the wire so as to cause precipitation or clotting of the fibers as deposited on the wire from the head box, by either shocking or dilution.

For the purpose of illustration, the invention will further be described in connection with the accompanying drawing which diagrammatically illustrates the Fourdrinier screen section of a paper-making apparatus, and particularly illustrates methods and means in connection therewith for washing the Fourdrinier wire with water-containing dispersing agent in accordance with the present invention.

Referring to the drawing, a dilute slurry of dispersed and individualized asbestos is supplied from the stock chest 10 to the head box 11 wherefrom it is picked up onto the Fourdrinier wire 12 by means of the suction formation roll 13. The Fourdrinier wire in conventional manner passes over the vacuum boxes 14 and the felted asbestos web on the wire 12 is transferred therefrom as it passes over the drive roll 15 by means of the pick-up felt 16 as the latter passes over the suction pick-up roll 17. The felt 16 is thereafter transferred from the web to drying means (not shown), such as, for example, a Yankee dryer.

The white water from the drainage trays 18 and 19 may be collected through line 20 and valve 21 to the white water tank 22 together with white water collected from the suction formation roll 13, vacuum boxes 14 and suction pick-up roll 17 by means of pump 23 and line 24. This white water may in whole or part be returned for use as make-up liquid through the pump 25, line 26, valve 27 and line 28 which may lead to suitable stock preparation tanks, or, in the alternative, if desired, discharged.

As is conventional, the Fourdrinier wire 12 in its lower return run as it passes over rolls 29 is subjected to washing to clean the wire by removing accumulations thereon. As previously described and in accordance with the present invention, washing of the Fourdrinier wire on its return run is accomplished by means of water containing asbestos dispersing agent. In accordance with the preferred embodiment of the present invention, such dispersing agent-containing water is the white water recovered as hereinbefore described. Thus, all or part of the white water from line 26 may be directed through valve 30

and line 31 to white water filter chest 32. This filter chest may, as illustrated, be a cylinder or decker type of save-all employing a wire-covered cylinder. The filtered white water is removed therefrom through line 33, valve 34 and pump 35 and delivered through line 36 to the screen spray 37.

As an alternative, I may employ a fresh aqueous solution containing a requisite amount of asbestos dispersing agent, supplied from the tank 38 by means of line 39 and valve 40 through pump 35 and line 36 to spray 37. In such case, the asbestos dispersing agent need not necessarily be the same one contained in the fiber dispersion, but still one, or a mixture of asbestos dispersing agent, as described in my aforesaid co-pending application, capable of protecting the asbestos fibers from clotting. If desired, the solution collecting in the pan 19 may be discharged therefrom through line 12, valve 41 and line 42. As a further alternative, instead of discharging the solution from line 42 to waste, the discharge from line 42 may be recovered for use as slurry make-up or, as a further alternative, the discharge from line 42 may be directed by means, not shown, to tank 38 for direct recirculation thereof.

It will thus be seen that by proceeding in accordance with the preferred method, that is, by employing the white water recovered in the usual manner as the solution for washing the screen, an adequate amount of dispersing agent in the wash water will already be present since such amount was present in the slurry water for maintaining the dispersion, and in commercial practice the dispersing agent is generally contained therein in excess so as to have insured stability of the original dispersion.

As further indicated from the foregoing, if desired, wash water may be employed which is not necessarily recovered white water. In such instance, the wash solution should contain an adequate amount of dispersing agent, such as will not cause precipitation of fibers and entanglement thereof on the screen, the amount being related to the character of the agent employed as hereinbefore pointed out. In the event the agent employed in this wash water solution is the same as the agent employed in preparing the original dispersion, it may be combined with the wash water. In the alternative, that is to say, for example, if the dispersing agent employed in the wash water is other than the agent employed in preparing the original asbestos dispersion, it may be wasted after use or recirculated in a separate but continuous wash system, as hereinbefore described in accordance with the description of the apparatus.

Although I have particularly described the present improvement in connection with the washing of a Fourdrinier screen, it will be understood that my invention is of like effect in respect to other endless forming or conveying surfaces employed in paper-making machines which are intermittently or continuously washed. That is to say, washing operations of surfaces on which my individualized and dispersed asbestos fibers are deposited prior to drying should not be washed with clear water, or water deficient in an amount of dispersing agent adequate to maintain the fibers in their desired dispersed individualized condition.

I claim as my invention:

1. A method which comprises forming a fibrous asbestos web from an aqueous alkaline colloidal dispersion of individualized chrysotile asbestos

fibers containing organic chrysotile asbestos colloidizing agent both adsorbed on the fibers and in the aqueous phase maintaining said dispersion, upon an endless continuously moving foraminated surface, continuously stripping the formed web therefrom, and washing said surface, after removal of the web, with an aqueous dispersion-maintaining solution of asbestos colloidizing agent.

2. A method which comprises forming a fibrous asbestos web from an aqueous alkaline colloidal dispersion of individualized chrysotile asbestos fibers containing organic chrysotile asbestos colloidizing agent both adsorbed on the fibers and in the aqueous phase maintaining said dispersion, upon an endless continuously moving foraminated surface, continuously stripping the formed web therefrom, and washing said surface after removal of the web with a fresh aqueous solution of said colloidizing agent of a concentration substantially equal to that of the aqueous phase of said dispersion.

3. A method which comprises forming a fibrous asbestos web from an aqueous alkaline colloidal dispersion of individualized chrysotile asbestos fibers containing organic chrysotile asbestos colloidizing agent both adsorbed on the fibers and in the aqueous phase maintaining said dispersion, upon an endless continuously moving foraminated surface, continuously stripping the formed web therefrom, and washing said surface after removal of the web, with white water containing said colloidizing agent recovered in the process.

4. A method which comprises forming a fibrous asbestos web from an aqueous colloidal asbestos dispersion of individualized colloidal asbestos fibers containing organic chrysotile asbestos colloidizing agent both adsorbed on the fibers and in the aqueous phase maintaining said dispersion, upon an endless continuously moving foram-

inated surface, continuously stripping the formed web therefrom, collecting colloidizing agent-containing white water separated in the process and filtering same, and washing said foraminated surface, after removal of the web therefrom, with said filtered white water.

5. In a method of making a fibrous asbestos web wherein an aqueous alkaline colloidal dispersion of individualized chrysotile asbestos fibers containing organic chrysotile asbestos colloidizing agent both adsorbed on the fibers and in the aqueous phase maintaining said dispersion, is deposited on an endless continuously moving foraminated surface and the excess aqueous solution removed therefrom through said surface to form a fibrous web thereon, the improvement which comprises collecting and filtering a portion of said aqueous solution and washing said foraminated surface therewith in the path of its return travel.

#### References Cited in the file of this patent

##### UNITED STATES PATENTS

| Number    | Name         | Date          |
|-----------|--------------|---------------|
| 1,302,313 | Coppage      | Apr. 29, 1919 |
| 1,907,616 | Tucker       | May 9, 1933   |
| 2,068,219 | Badollet     | Jan. 19, 1937 |
| 2,182,274 | Baker et al. | Dec. 5, 1939  |
| 2,217,005 | Clapp        | Oct. 8, 1940  |
| 2,220,386 | Badollet     | Nov. 5, 1940  |

##### FOREIGN PATENTS

| Number  | Country       | Date          |
|---------|---------------|---------------|
| 481,705 | Great Britain | Mar. 16, 1938 |

##### OTHER REFERENCES

Chemistry of Pulp and Paper Making by Sutermister, 3rd Ed. (1941), pgs. 407-411, pub. by John Wiley and Sons, New York.

40 Morrison, Paper Industry and Paper World, May 1943, p. 192.